

## UNITED STATES PATENT OFFICE.

HENRY T. CHANDLER, OF DETROIT, MICHIGAN.

## ALLOY STEEL.

No Drawing.

Application filed August 19, 1918. Serial No. 250,477.

*To all whom it may concern:*

Be it known that I, HENRY T. CHANDLER, a citizen of the United States, and residing at Detroit, in the county of Wayne and State of Michigan, have invented a new and Improved Alloy Steel, of which the following is a specification.

The present invention has reference to new alloy steels, its object being to provide 10 a heat treated steel or alloy steel which possesses physical properties and combinations of properties of a relatively high order as compared with the best practice in steels heretofore. Certain forms of these steels 15 are especially adapted for armor plate, but the steels may be used for other purposes, in fact, they may be advantageously substituted generally for those steels or steel alloys wherein high values of static or dynamic 20 physical properties or combinations of these properties enter as determining factors. In these new steels, these properties are not only in themselves of the highest order, but there may be associated with them by suitable 25 heat treatment a high degree of hardness as measured by the Brinell, scleroscope and scratch tests which renders the steel particularly suitable for armor plate, projectiles and guns, and also gears and the like.

The nature and objects of my invention may be exemplified by considering its application to armor plate, for the requirements and service to be met by such material is such that only the best products of the steel makers' art can be used, and, obviously a new steel which meets the requirements of this particular class of service will also, with modifications apparent to those 40 skilled in the art, be of value in general application for other uses such as tools, dies and other machine parts in some of which the question of extreme toughness, rather than toughness associated with extreme 45 hardness, is more nearly controlling.

Due to the recent developments of guns, ammunition and methods of warfare, these service requirements of armor plate have so increased that they can be met generally 50 only by the best high duty steels under ideal

conditions of manufacture and heat treatment; and for some purposes—as in the case of a suitable protection for the vital parts of an aeroplane and in body armor, for example—where weight may be said to be the 55 determining factor, cannot be met satisfactorily at all. Under these conditions, requiring super-excellent physical properties and combinations of such properties, the various alloy steels generally employed for 60 this purpose, namely, the nickel steels, the nickel chromium steels and the silico-manganese steels as well as the later developed nickel—chromium—cobalt, molybdenum and manganese-nickel-vanadium steels, are subject to a high percentage of loss both in the 65 process of manufacture and on ballistic test, which has been with the best manufacturing practice heretofore seldom under 15% and usually from 30% to 60%. In other words, 70 they are sensitive to the various steps involved in their manufacture, particularly in the matter of heat treatment, the result being that plates produced in substantially the same way, within the limits of manufacturing practice, often differ sufficiently from others to be rejected. This is particularly 75 true in the case of thin sheets, which are generally used for mobile instruments.

The capability of a steel to resist the impact of projectiles is dependent upon a variety of elements among which hardness and toughness stand out. These two properties may be regarded as antagonistic to each other, in other words, steels possessing a 80 high degree of hardness, either Scleroscope or Brinell, are not ordinarily tough and those unusually tough are of the softer grades. For example, a plate of extreme hardness becomes brittle and cracks or 85 breaks upon receiving the impact of the projectile, while a soft tough plate is too readily pierced. To properly resist the impact of the projectile, the face of the plate must be so hard as to shatter the former and thus 90 spread its blow over a considerable area, for without this shattering action the thickness of the metal required to withstand the projectile proves too great for most uses. In addition, a high degree of toughness, of 95

which high breaking strength, increased elongation and high reduction in area before breaking are evidence, is necessary, as the entire energy of the blow must be absorbed by the plate without it cracking or punching through.

The best steels heretofore employed for armor plate, even when carbonized or surface hardened, have for any given service a very narrow range of hardness within which they possess the required toughness, and departures from these limits have led to cracking and breaking if above or piercing if below. This hardness is dependent upon heat treatment, and the latter, being difficult to control accurately, is largely responsible for the high ballistic loss.

Because of the non-uniformity of product, in so far as its suitability for use as armor plate is concerned, resulting from present practice, it is customary to submit each plate (up to a thickness of substantially .6 of an inch, and representative samples of thicker material) to a firing or ballistic test, which consists in firing, with a standard rifle or machine gun, bullets of the regular or of the armor piercing type at predetermined ranges and velocities, depending upon the service for which the plate is intended. Such plates as withstand the impact of the projectiles without breaking, cracking or undue deformation are accepted as satisfactory, while those pierced, cracked or broken are rejected. For example, a satisfactory plate, .615 inches in thickness should, under present testing practice, withstand at a range of 50 yards, five shots, within the area of a five inch circle, fired from a standard machine gun calibre .30 with armor piercing bullets having a muzzle velocity of 2800 feet per second.

The usual steels have also proven, for the most part, difficult to manipulate in one or more of the melting, casting, heat treatment and forming operations necessary in their manufacture. Neither has it been possible to produce a steel of appreciably less thickness and capable of withstanding the test outlined above.

To recapitulate: The determining factors in the production of satisfactory armor plate are—

1. Ability to withstand bullets or other projectiles without penetration or fracture, that is, high ballistic yield.
2. Weight, which is, of course, a prime consideration needing no explanation.
3. Ease of manufacture under present steel making methods.
4. Cost, which materially enters into the three above named considerations; and these same factors enter to a greater or less degree into the production of high class steels for use generally in various arts of which the automotive and machine building industries are good examples. That is, my invention,

as hereinafter pointed out, although supplying armor plate of the highest grade, is also applicable under modified analyses and heat treatment to the softer classes of steels such as are commonly used in the manufacture of machine parts such as crank shafts and the like.

By my invention, I am enabled to produce a steel which may be termed a zirconium steel, which is characterized by possessing, in a marked degree, physical properties and combinations of properties such as hereinbefore set forth, of an excellence which has hitherto seldom been attained in the fabrication of steel and steel products. 70 In carrying out my invention I add zirconium to the usual elements constituting what is usually termed steel, as determined by the requirements of the particular field of use, in quantities at least sufficient to 75 produce a product containing zirconium from a substantial fraction of one-tenth of one per cent to not materially more than one per cent, altho for certain special purposes it may be desirable to carry the percentage higher. These percentages appear to be notably low, but the presence of zirconium in the finished product under conditions which I will point out even in extremely small quantities, such as .04 to .08 of 80 one per cent, produces marked effects as will appear.

In the periodic system of classification of the elements, zirconium is placed in the group containing carbon, silicon and titanium, indicating that it possesses chemical and hence metallurgical properties and characteristics similar to those of these elements. I am aware that it has been suggested, as for example in the United States Letters Patent 105 by Weiss No. 982,326, to use zirconium in the manufacture of castings and the like as a deoxidizing substance adapted to produce sound castings, in which respect zirconium has an action closely akin to that of titanium; and that as thus employed it has the effect of increasing certain of the properties of the metal as might be expected from the use of any satisfactory deoxidizing agent. I do not, however, propose to make use of those deoxidizing characteristics which may be described as being analogous to titanium, but to take advantage of those characteristics which may be described as being analogous to those of carbon and silicon. Steels produced by my invention are true zirconium steels in contrast with steels merely deoxidized by that element and which might contain small amounts of zirconium included in the metal as an inert slag. For example: In certain classes of my steels one effect of the added zirconium will in the annealed or normalized state be evidenced a microscopically visible change in the appearance of the nor- 110 115 120 125 130

mal pearlite. The zirconium in this type of steel behaves in a manner similar to carbon; in other types the element remains substantially in solid solution and affects the properties of the steel indirectly, when its action is comparable to the behavior of silicon. In other words, in some cases I replace part of the carbon of the usual steels by zirconium and thereby secure after proper heat treatment a steel possessing a combination of physical properties well in advance of those of the corresponding carbon steel; likewise in other cases, I replace part or all of the silicon by zirconium and by heat treatment obtain a zirconium steel or a zirconium-silicon steel having a combination of the special properties of silicon steels and individually in excess thereof without the corresponding difficulties involved in the corresponding increase in silicon. These zirconium steels therefore have advantages over the corresponding silicon steels both in the matter of ultimate physical properties and in various steps involved in manufacture and production.

I add the zirconium in a form which is soluble in the liquid and either partially or wholly soluble in the solid state of the steel, and for this purpose I prefer to employ an alloy or compound of zirconium, low in carbon, together with iron, nickel, cobalt, copper, silicon, magnesium, aluminum, manganese, or titanium either singly or in combination, which contains comparatively large percentages of zirconium. It is desirable that an element having a greater chemical affinity for oxygen, such as aluminum or magnesium, be present in the alloy for by this means complete deoxidation of the steel is effected without a corresponding loss of zirconium. If the steel to be produced is to be of the tungsten, chromium, molybdenum or vanadium types, the zirconium alloy may contain the required amounts of these elements with advantages as they increase the specific gravity and somewhat aid the absorption of the corresponding alloy by the steel.

I have found the following alloys to successfully serve the purpose:

|    |       |       |       |       |
|----|-------|-------|-------|-------|
| Zr | 11.64 | 18.62 | 43.57 | 17.44 |
| Fe | 70.72 | 65.03 | 28.30 | 1.32  |
| Si | 13.54 | 10.87 | 13.29 | 6.64  |
| Al | 1.88  | 4.08  | 12.72 | 6.12  |
| Cr | 0.30  |       |       |       |
| Ti | 1.25  | .50   | .55   |       |
| C  | 0.21  | 0.37  | .33   | .50   |
| Ni |       |       | 65.30 |       |
| W  |       |       | 1.70  |       |

Such alloys may be made by the Goldschmidt reaction or reduced in the electric furnace, or a combination of these methods may be used.

The amount of the alloy to be added in order to secure the required percentage of

zirconium is dependent upon its analysis and the analysis, temperature, and state of deoxidation of the steel. For example, alloys high in aluminum are lighter than the molten steel and it is difficult to effect their complete solution, and alloys containing a high percentage of carbon tend to slag off part of the zirconium carbide. A badly oxidized steel bath will slag off the zirconium as zirconium-oxide. I prefer to add the zirconium in the furnace just previous to pouring the steel, after deoxidation and under a neutral or slightly acid slag. Zirconium alloys of low melting point, such as the nickel-silicon types, may be added in the ladle.

The specific effects of the presence of zirconium on the properties of steel is illustrated in the following comparative tables. Especially are they to be derived when the zirconium is used in combination with nickel, and I have chosen steels of this type as examples for purposes of illustration. These four steels were all poured from the same heat of steel by successively tapping the furnace after increasing zirconium additions. The ingots were forged and the test bars from them were heat treated under as nearly like conditions as possible.

#### Analyses.

(Iron in each instance forming balance of the 100%).

|    | No. 1.    | No. 2.    | No. 3.    | No. 4.    | 100 |
|----|-----------|-----------|-----------|-----------|-----|
|    | Per cent. | Per cent. | Per cent. | Per cent. |     |
| C  | .36       | .36       | .45       | .45       |     |
| Ni | 2.86      | 2.81      | 2.74      | 2.66      |     |
| Si | 1.25      | .82       | 1.21      | 1.65      |     |
| Zr | 0.00      | 0.22      | 0.33      | 0.30      |     |
| Mn | .62       | .67       | .68       | .73       |     |
| S  | .027      | .018      | .018      | .016      |     |
| P  | .014      | .018      | .018      | .016      | 105 |

Heat treatment—size of sample treated, 6" x 7/8" round.

- (1) 1650 degrees F., up to heat, cool in mica.
- (2) 1560 degrees F., hold at temperature 110 10 minutes, quench in oil.
- (3) 880 degrees F., hold at temperature 2 hours, air cool.

Standard test bars of .505" diam. were 115 made and tested with the following results:

#### Physical properties.

|                  | No. 1.  | No. 2.  | No. 3.  | No. 4.  | 120 |
|------------------|---------|---------|---------|---------|-----|
|                  |         |         |         |         |     |
| Tens. str.       | 266,000 | 280,000 | 310,000 | 307,000 |     |
| Elastic limit.   | 260,000 | 251,000 | 270,000 | 264,000 |     |
| Red area.        | 36.2%   | 45.3%   | 42.0%   | 35.0%   |     |
| Elongation on 2" | 11.5%   | 18.0%   | 13.5%   | 12.5%   |     |
| Brinell.         | 512     | 512     | 532     | 555     |     |
| Sclerometer.     | 70      | 78      | 80      | 84      | 125 |

Steel of the type shown by the analysis of ingot #1 above, though containing no zirconium, is in itself an excellent material for armor plate, and as such has found wide 130

use. The marked betterment of all the physical properties produced by the presence of the zirconium is therefore of great benefit to the manufacturer for it permits 5 him a wider range of manufacturing practice without exceeding the limits of hardness and toughness required and hence a greater manufacturing and ballistic yield.

Attention is especially called to the extremely high reduction in area corresponding with the tensile strength and hardness of bars #2 and #3. It will be observed that the product of the mean breaking strength and the elongation taken together 15 with the small mass of steel effected by breaking as indicated by the high reduction in area is extremely high for the hardness indicated. This may be called the merit number of the steel as it indicates the amount of work necessary to be done on a 20 unit mass of the steel to cause breaking, and is a factor of prime importance in armor plate, springs, dies, and the like.

The results obtained in armor plate steel 25 produced in accordance with my invention is illustrated in the following silico-nickel manganese steel in which part of the silicon is replaced by the element zirconium; a plate seven inches in diameter and having 30 an average thickness of .34 inch was forged from a steel of the following analysis:

|                          |       |
|--------------------------|-------|
| Carbon                   | 0.38  |
| Nickel                   | 3.20  |
| Silicon                  | 0.88  |
| Manganese                | 0.75  |
| Zirconium                | 0.16  |
| Sulphur                  | 0.033 |
| Phosphorus               | 0.018 |
| Iron—balance of the 100% |       |

It was then heated to 1600 degrees F. and cooled in mica dust, reheated to 1560 degrees F., which is slightly beyond the critical range and quenched in oil and finally drawn at 375 degrees F. for two hours. This treatment yielded a fine martensitic structure.

The nature and results of the ballistic 50 test of the above mentioned plate are tabulated below.

| No. | Range, yards. | Rifle.         | Muzzle velocity, f. s. | Bullet.                         | Caliber. |
|-----|---------------|----------------|------------------------|---------------------------------|----------|
| 1   | 50            | Springfield    | 2300                   | Regulation cupro-nickel jacket. | .30      |
| 2   | 50            | Springfield    | 2300                   | Clay A.P.                       | .30      |
| 3   | 10            | Springfield    | 2300                   | Clay A.P.                       | .30      |
| 4   | 10            | Special Newton | 3200                   | Clay A.P.                       | .30      |
| 5   | 10            | Special Newton | 3200                   | Clay A.P.                       | .30      |

In all the above the line of fire was at right angles to the surface of the plate. The plate resisted all shots without penetration or fracture. A slight indentation was 65 caused by the cutting action of the projec-

tile and in the case of shots number four and number five the plate slightly bulged at the point of impact.

It will be seen that the plate, altho approximately only one half the regulation .65" thickness which is permitted under these conditions, withstood under standard conditions the firing of a gun having a muzzle velocity and consequently an impacting force far greater than that of the gun used in standard testing practice. This advance 75 not only meets the requirements for armor plate intended for ordinary uses, but also provides a weight and strength adapted for the needs of aeroplane protection, for body armor and for the protection of light, mobile implements generally.

Physical tests on bars cut from this plate gave the following results:

|                      |            |
|----------------------|------------|
| Brinnell hardness    | 578        |
| Selerescope hardness | 78.85      |
| Tensile strength     | 286,000    |
| Elastic limit        | 280,000    |
| Red in area          | 35%        |
| Elongation           | 10.5%      |
| Angle of cold bend   | 25 degrees |
| Specimen .34"        | 60"-6"     |

The above physical properties afford the explanation of the results noted on the ballistic test. It will be observed that the hardness was sufficient when coupled with the elastic limit, to shatter the projectile; the toughness, as measured by the mean breaking strength and the reduction in area, was sufficient to prevent the local punching out (important consideration in thin plate); and the toughness, as measured by the elongation and mean breaking strength and indicated by the angle of cold bend, was sufficient to prevent fracture and breaking.

For armor plate up to .65 inch in thickness I prefer the following analysis:

|               |           |
|---------------|-----------|
| Carbon        | 38-46     |
| Nickel        | 2.72-3.50 |
| Silicon       | 1.20-1.50 |
| Zirconium     | 10-40     |
| Manganese     | 80-1.00   |
| Sulphur       | 035 max.  |
| Phosphorous   | 035 max.  |
| Balance iron. |           |

For thicker plates the addition of .30% molybdenum or its equivalent in chromium or tungsten or approximately .35% cobalt is desirable to increase the hardening properties. Two tenths of one per cent vanadium may also be added with advantage. Such a steel is readily capable of rolling into thin sheets (e. g. .20" 0 and gives excellent properties upon oil hardening).

While the examples given only illustrate the effect of zirconium on a silicon steel, nevertheless its similarity to carbon is such that it may be substituted in small quan-

tities for that element, as for example in the chrome steels and chrome nickel steels, with results similar to those given. Furthermore, such zirconium steels may be modified by 5 the additions of molybdenum, cobalt, tungsten, vanadium and other alloys to increase certain of their physical properties for special uses in a manner familiar to those skilled in the art.

10 The above examples illustrate the properties obtainable in steels of the hard type, suitable for armor plate, springs, gears, dies and other machine parts requiring no machining operations other than grinding after 15 the heat treatment. However, with suitable modifications in analysis and heat-treatment, such as the use of smaller percentage of carbon and higher drawing temperatures, steels of the softer and more readily 20 machinable types may be produced and, because of the excellence of their physical properties, ready workability and cost of manufacture are especially suitable for general forgings for machine parts such as 25 crankshafts, axles, connecting rods and the like.

For example: a steel of the following analysis—

|               | Per cent. |
|---------------|-----------|
| 30 C          | 32        |
| Mn            | 75        |
| Si            | 80        |
| Ni            | 2.75      |
| S             | 018       |
| 35 P          | 020       |
| Zr            | 22        |
| Iron—balance. |           |

when heat treated as follows on a 1" section: 40 (1) 1600 degrees F. air cool; (2) 1560 degrees F. up to heat 10 minutes, quench in oil; (3) 1050 degrees F. anneal 2 hrs. gave the following physical properties:

|                     |                          |
|---------------------|--------------------------|
| 45 Tensile strength | 156,000 lbs. per sq. in. |
| Elastic limit       | 155,200 lbs. per sq. in. |
| Elongation          | 17%                      |
| Red. area           | 54%                      |
| Brinnell            | 302%                     |

50 As hereofore pointed out, various changes in the analyses and heat treatments involved may be made by those skilled in the art, for the purpose of producing modified 55 commercial steels of the types rendered available through my invention, and I do not, therefore, wish to be limited except as indicated by the subjoined claims.

Owing to the small percentages used and 60 the comparative abundance and cheapness, zirconium steels of extraordinary quality may be manufactured according to my invention at a far less cost than by means of the usual alloys employed in steel manufacture such as vanadium, tungsten, etc.

I claim:—

1. Heat treated alloy steel including the usual constituents that go to make up steel and less than one per cent of zirconium as an added element. 70

2. A steel containing zirconium as an added element and characterized in the finished state by a substantially solid solution of zirconium pearlite which appears with the usual pearlite or ferrite in the steel 75 in the annealed state.

3. Heat treated alloy steel containing less than one per cent of zirconium.

4. Alloy steel including the usual constituents that go to make up steel and embodying zirconium in an amount between substantially one tenth of one per cent by weight and substantially one per cent by weight. 80

5. Heat treated alloy steel suitable for 85 use in thin sheets as armor plate and having a high ballistic yield when so applied, and embodying zirconium in quantities between .04 per cent and substantially one per cent by weight. 90

6. A steel for producing articles to be heat treated, said steel containing zirconium as an added element and being characterized in the annealed or normalized state by microscopically visible zirconium eutectic 95 or pearlite.

7. Steel embodying less than one per cent of zirconium which steel has been heated to within the critical range.

8. In the manufacture of steel, the addition of zirconium in a form which is soluble in the metal in the liquid state and partly or wholly soluble in the metal in the solid state. 100

9. In the manufacture of steel, the addition of zirconium in a state which will form a zirconium compound which is soluble in the metal in the liquid state and wholly or partly soluble in the metal in the solid state. 105

10. A heat treated steel in which a part of the carbon is replaced by less than one per cent of the element zirconium.

11. Armor plate including the usual constituents that go to make up steel and embodying zirconium as an added element up to one per cent. 115

12. Armor plate having a high ballistic yield and containing the usual constituents that go to make up steel and embodying zirconium as an added element in quantities ranging from .04 per cent to substantially one per cent by weight. 120

13. A commercial steel having a maximum merit number at a relatively high degree of hardness and containing zirconium as an added element in quantities ranging from a fraction of one per cent to not substantially more than one per cent by weight. 125

14. A mechanically worked steel contain-

6  
ing the usual ingredients and zirconium as an added element in an effective amount up to substantially 1 per cent.

15. Forged alloy steel containing zirconium in an effective amount up to substantially 1%.

16. Steel embodying zirconium in an effective amount up to substantially 1%,

which steel has been mechanically worked while hot.

17. Alloy steel including the usual constituents that go to make up steel and embodying zirconium in an effective amount up to substantially 1%.

HENRY T. CHANDLER.